

# United States Patent

Guzzi et al.

[15] 3,692,833

[45] Sept. 19, 1972

## [54] PHOTOGRAPHIC COLOR COUPLERS

[72] Inventors: Alberto Guzzi, Viale Della Liberta; Remo Magagnoli, Via Gramsci, both of Ferrania, Italy

[22] Filed: Aug. 27, 1970

[21] Appl. No.: 67,569

### Related U.S. Application Data

[62] Division of Ser. No. 701,995, Jan. 31, 1968, Pat. No. 3,591,384.

### [30] Foreign Application Priority Data

Feb. 15, 1967 Italy.....34846 A/67

[52] U.S. Cl.....260/559 S

[51] Int. Cl.....C07c 103/30

[58] Field of Search.....260/559, 560

### [56] References Cited

### UNITED STATES PATENTS

3,591,384 7/1971 Guzzi et al.....96/100

Primary Examiner—Henry R. Jiles

Assistant Examiner—Harry I. Moatz

Attorney—Carpenter, Kinney & Coulter

[57]

### ABSTRACT

This invention relates to compounds useful as photographic couplers having the general formula:



wherein X is alkyl, Y is either carbonyl or sulfonyl, R is alkyl having from five to 20 carbon atoms and Z is hydrogen or halogen. The invention also relates to the use of the abovementioned compounds in photographic emulsions.

5 Claims, 2 Drawing Figures

PATENTED SEP 19 1972

3,692,833

FIG. 1



FIG. 2



INVENTORS  
ALBERTO GUZZI  
BY REMO MAGAGNOLI

Carpenter, Kinney & Coulter  
ATTORNEYS

1

## PHOTOGRAPHIC COLOR COUPLERS

This application is a division of application Ser. No. 701,995, now U.S. Pat. No. 3,591,384.

This invention relates to a class of couplers capable of forming stable cyan or blue-green dyes by color development in color photographic materials.

In the production of colored images by the color development of silver halide emulsion layers in a multi-layer film construction the image formed after light exposure of the reducible silver salts is developed in the presence of a coupler, i.e. a compound which reacts with the oxidation products of the color developer to form a dye. Cyan images are generally obtained by the formation of an indophenol dye from a 1-hydroxy-2naphthamide coupler. 15

One important requirement of color couplers used in color photography is the ability to resist bleeding or migration through and outside of the photographic emulsion layers in which they are contained. An effective means for solving the migration problem is provided by the dispersed coupler method, in which the coupler is dissolved in high boiling organic solvents, such as tricresyl phosphate or dibutyl phthalate, and the resulting solution is intimately dispersed throughout the silver halide emulsion. To obtain the best results in terms of the dispersion and photographic efficiency the solution of coupler in the organic solvent should be highly concentrated. Couplers which are highly soluble in or miscible with the organic solvent are therefore commonly selected for use in dispersed coupler systems. In general, couplers having a relatively low melting point are quite soluble in such organic solvents. However, it is also desirable to select couplers which produce dyes having good stability to light, heat

2



(1)



(2)



Table I shows some analytical data of these illustrative couplers, the analyses being made after only one crystallization of the raw reaction product. Included are their desirable melting points. Their high degree of solubility in organic solvents normally used for dispersing couplers in a gelatin emulsion permits the use of a solvent/coupler ratio far lower than 1.0 without any noticeable decrease in yield of dye.

TABLE I

| Coupler No. | Melting point<br>(° F.)        | O, percent |       | H, percent |       | N, percent |       | Cl, percent |       | —OH<br>percent<br>content<br>found | Crystalliza-<br>tion solvent |
|-------------|--------------------------------|------------|-------|------------|-------|------------|-------|-------------|-------|------------------------------------|------------------------------|
|             |                                | Found      | Calc. | Found      | Calc. | Found      | Calc. | Found       | Calc. |                                    |                              |
| 1.....      | { 215.6-219.2<br>(102-104° C.) | 78.46      | 78.39 | 8.28       | 8.11  | 3.00       | 3.04  | .....       | ..... | 99.27                              | Ethanol.                     |
| 2.....      | { 149.0-150.8<br>(65-66° C.)   | 72.55      | 72.9  | 7.25       | 7.3   | .....      | ..... | 7.16        | 7.17  | 98.81                              | Heptane.                     |
| 3.....      | { 208.4-210.2<br>(98-99° C.)   | .....      | ..... | .....      | ..... | .....      | ..... | .....       | ..... | 99.41                              | Acetic acid.                 |
| 4.....      | { 240.8-242.6<br>(116-117° C.) | .....      | ..... | .....      | ..... | 5.86       | 5.90  | 5.86        | 5.90  | 98.44                              | Do.                          |

and moisture and having good spectral characteristics, particularly low secondary absorptions.

It is an object of this invention to provide a new class of outstanding cyan couplers and photographic emulsions incorporating such couplers.

The cyan couplers of this invention have the formula:



wherein X is alkyl, preferably a lower alkyl ( $C_1$ — $C_6$ ), Y is either carbonyl or sulfonyl, R is  $C_5$ — $C_{20}$  alkyl, and Z is hydrogen or halogen, preferably chlorine or bromine. These couplers are easily obtained in a very high purity by methods described later.

Illustrative couples are as follows:

formed by normal color development procedures. For example, coupler (1) can be incorporated into a photographic emulsion with 1 part dibutyl phthalate containing 4 parts of coupler.

In addition to the abovementioned characteristics the claimed couplers react with N,N-dialkyl-p-phenylenediamine during color development to provide dyes which are particularly stable to light, heat and moisture. For example, if one of these couplers is dissolved in dibutyl phthalate, dispersed in a photographic emulsion, coated onto a transparent support, exposed and developed with diethyl-p-phenylenediamine, the resultant color shows no noticeable change in either color density or hue after exposure to a xenon lamp for 10 hours. Coated samples prepared in similar manner were exposed through a scale of decreasing densities, i.e. grey scale, and developed in color developer with excellent sensitometric results, even after storage for 24 hours at a temperature of 194.0°F. (90°C.) and a relative humidity of 75 percent. In FIG. 1 curve A is the sensitometric curve (read in red light) for coupler (1) and curve B is the sensitometric curve for coupler (1)

after 24 hours storage under the abovementioned conditions. These curves show the excellent stability of dyes prepared from the couplers of this invention.

The spectral absorption of the cyan dyes obtained from these couplers and N,N-dialkyl-p-phenylenediamine developers make them particularly suitable for preparing color negative materials. Furthermore, they have a low absorption in the green portion of the spectrum, which is very desirable. In FIG. 2 an illustrative comparison of the spectral absorption of N,N-diethyl-p-phenylenediamine developed couplers in dibutyl phthalate, absorption curve A being that of abovementioned coupler (3) and absorption curve B being that of a coupler of the formula:



The coupler of curve B is a known coupler having some structural similarity to the couplers of this invention. From a comparison of curves A and B it is apparent that curve A represents lower absorption in the 500 and 600 millimicron region than curve B.

The couplers of the present invention can be prepared by reacting the suitable amines with 1-hydroxy-2-naphthoic acid or 1-hydroxy-4-halo-2-naphthoic acid derivatives, such as their phenyl esters. In particular, the preparations of some couplers of said class were carried out in the following way:

a. Preparation of 4-methyllaurophenone

Into a 500 ml. flask containing a suspension of 59 g. of  $\text{AlCl}_3$  in 168 ml. of dry toluene, 69.2 g. of lauroyl chloride were rather quickly introduced. The temperature rose to 140.0°F. (60°C.). The mixture was kept under stirring at a temperature of 176.0°F. (80°C.) for 22 hours, then was poured with vigorous stirring into 1,000 ml. of water and 66.5 ml. of concentrated hydrochloric acid. After about one hour the organic layer was removed and washed, first with a 1%  $\text{Na}_2\text{CO}_3$  solution and then with water. The toluene solution was then dried with calcium chloride, and the solvent was removed under vacuum. The residue, consisting of a readily solidifying oil, was crystallized from ethanol. Yield: 58.8 g. (67 percent). M.p.: 113.0°-115.5°F. (45°-46.5°C.) Analysis: for  $\text{C}_{19}\text{H}_{30}\text{O}$  calculated: C% 83.57; H% 10.94 found: C% 83.27; H% 10.94.

b. Preparation of 3-nitro-4-methyllaurophenone

In a beaker provided with stirrer and thermometer, was placed 190 ml. of  $\text{HNO}_3$  (D-1.52) and then 69.9 g. of 4-methyllaurophenone was added in increments. The operation was carried out as rapidly as possible while maintaining the reaction temperature below 44.6°F. (7°C.). After completion of the ketone addition the mixture was stirred for an additional 5 minutes and then the mixture was added dropwise into 1 liter of ice water. The precipitated product was filtered off and thoroughly washed with water, then allowed to dry in the air. By crystallization from methanol 86.4 g. (70 percent) of the nitro derivative with M.p.: 122.0°-123.8°F. (50°-51°C.) was obtained.

c. Preparation of 3-amino-4-methyllaurophenone

56.4 g. of 3-nitro-4-methyllaurophenone was dissolved in a boiling mixture of 530 ml. of 90 percent acetic acid and 260 ml. of ethanol. Then 106 g. of iron powder was slowly added. After completion of the addition boiling was continued for about 30 minutes, after which the ferrous slime was hot filtered and the filtrate was poured with stirring into 17.5 ml. of water. The amine which separated was filtered off and thoroughly washed with water. Yield of raw product: 48.6 g. By crystallizing the raw product from 485 ml. of ethanol and decolorizing with charcoal, 41.5 g. (81.2 percent) of product having a M.p. of 167.0°-170.6°F. (75°-77°C.) was obtained. Analysis: for  $\text{C}_{19}\text{H}_{31}\text{NO}$  calculated: N% 4.84; found: N% 4.65; —NH<sub>2</sub> content: 100.00 percent.

d. Preparation of 1-hydroxy-2-(2'-methyl-5'-lauroyl)naphthanilide (Coupler 1)

In a Claisen flask arranged for distillation under 20 vacuum a mixture of 63.6 g. of 3-amino-4-methyllaurophenone and 63.6 g. of phenyl 1-hydroxy-2-naphthoate was melted. At this point vacuum was applied in order to remove the phenol which was liberated as the reaction continued. After about half an 25 hour the amount of distilled phenol was 22 g. (theory: 22.6 g.). The residue was crystallized from ethanol. Yield of coupler: 91.5 g.

e. Preparation of 1-hydroxy-4-chloro-2-(2'-methyl-5'-lauroyl)-naphthanilide (Coupler 2)

30 By working in the same way as described for the coupler 1 and employing an equivalent amount of phenyl 1-hydroxy-4-chloro-2-naphthoate instead of phenyl 1-hydroxy-2-naphthoate 86 g. of coupler was obtained after crystallization from heptane.

f. Preparation of p-tolyl cetyl sulfone

35 Into a reaction flask 75 g. of sodium p-toluenesulfinate tetrahydrate, 300 ml. of ethanol and 91.5 g. of cetyl bromide were introduced. The mixture was heated at reflux on a water bath for 24 hours and was then diluted with 1 liter of water. A white precipitate was obtained which, after being filtered, washed and dried, was purified by crystallization from ethanol. Yield: 82.1 g. M.p.: 154.4°-156.2°F. (68°-69°C.) Analysis: for  $\text{C}_{23}\text{H}_{40}\text{O}_2\text{S}$  calculated: C% 72.57; H% 10.5; S% 8.4; found: C% 72.36; H% 10.4; S% 8.28.

g. Preparation of 3-nitro-4-methylphenyl cetyl sulfone

40 It was obtained in a way similar to the 3-nitro-4-methyllaurophenone by using 112 ml. of fuming  $\text{HNO}_3$  for 56.8 g. of p-tolyl cetyl sulfone. Yield: 55.2 g. (from ethanol) M.p.: 161.6°-163.4°F. (72°-73°C.).

h. Preparation of 3-amino-4-methylphenyl cetyl sulfone

45 Prepared in a way similar to the 3-amino-4-methyl-laurophenone, it was crystallized from ethanol. M.p.: 140.0°-41.8°F. (60°-61°C.) Analysis: NH<sub>2</sub>% content 98.27.

i. Preparation of 1-hydroxy-2-(2'-methyl-5'-cetyl sulfonyl)-naphthanilide (Coupler 3)

50 By following the same procedure as the Coupler (1), 47.3 g. of 3-amino-4-methylphenyl cetyl sulfone was reacted with 34.7 g. of phenyl 1-hydroxy-2-naphthoate. 59.2 g. of Coupler (3) was obtained.

j. Preparation of 1-hydroxy-4-chloro-2-(2'-methyl-5'-cetyl sulfonyl)-naphthanilide (Coupler 4)

55 The product was obtained by procedures similar to those used in the preceding examples from 39.5 g. of 3-



UNITED STATES PATENT OFFICE  
CERTIFICATE OF CORRECTION

Patent No. 3,692,833 Dated September 19, 1972

Inventor(s) Alberto Guzzi and Remo Magagnoli

It is certified that error appears in the above-identified patent and that said Letters Patent are hereby corrected as shown below:

Column 1, line 36, Table I, "0, percent" should be  
--C, percent--.

Signed and sealed this 29th day of May 1973.

(SEAL)

Attest:

EDWARD M. FLETCHER, JR.  
Attesting Officer

ROBERT GOTTSCHALK  
Commissioner of Patents